# EUROPEAN PATENT SPECIFICATION

(11) **EP 0 054 405 B1**
(45) Date of publication and mention of the grant of the patent: **13.02.1985**
(21) Application number: 81305807.0
(22) Date of filing: 09.12.1981
(51) Int. Cl.: D21H 5/00, B41M 1/36, B41M 7/00, B44C 5/04

(54) **Process for the manufacture of decorative laminates**
Verfahren zur Herstellung von Dekorationsschichtstoffen
Procédé pour la préparation de stratifiés décoratifs

(30) Priority: 12.12.1980 GB 8039933
(43) Date of publication of application: 23.06.1982
(73) Proprietor: Devon Valley Industries Limited, London W1N 9AF (GB)
(72) Inventor: Newman, John Allen Sandys, Honiton Devon (GB); Ritchie, Alison Mary, Lincoln (GB)
(74) Representative: Lyons, Andrew John

## Description

This invention relates to a process for the manufacture of decorative laminates, to the laminates so made and to a paper for use in the process.

Decorative laminates are used, for example, for surfacing furniture, particularly kitchen or other furniture where it is desirable to have a water- resistant, easily-wipeable surface, for counter tops in shops and cafes and for building panels. They may be white or coloured, and may be plain or printed, for example with a woodgrain or other pattern. Printing may be in several colours, and is usually effected by a rotogravure technique.

One well-known type of decorative laminate (usually known as a high-pressure laminate) consists of several so-called core sheets for imparting strength to the laminate, a decorative sheet serving to mask the uppermost core sheet and to afford the laminate an attractive surface, and an overlay sheet on top of the decorative sheet (the overlay sheet becomes transparent during manufacture of the laminate, and so does not mask the decorative sheet). A so-called barrier sheet can be provided between the decorative sheet and the uppermost core sheet to afford an additional masking effect. All the sheets forming the laminate are impregnated with a thermo-setting resin, for example a phenolic resin or a melamine- formaldehyde or other aminoplast resin (the various sheets making up the laminate are not usually all impregnated with the same resin). The impregnating resin in the case of the decorative sheet is most commonly a melamine formaldehyde resin. In the final impregnated sheet, the resin is usually present in an amount of the order of 100% w/w.

If the decorative laminate is to be of a printed design, the decorative sheet normally carries the print. Alternatively, however, the overlay sheet may carry the print on its surface which contacts the decorative sheet.

The core sheets are normally of strong, relatively inexpensive paper, for example unbleached softwood kraft paper. Such paper is not of uniform or particularly attractive appearance, and is not suitable for high quality printing. For this reason, it is necessary for the decorative sheet to be sufficiently opaque to mask the unattractive and non-uniform appearance of the uppermost core sheet, and for it to be suitable for high quality printing.

In another type of decorative laminate (usually known as a low-pressure laminate), a sheet of chipboard or similar material is used directly as a support for the decorative sheet, instead of the core sheets. The decorative sheet in such a laminate serves to mask the chipboard rather than the core sheets. Again, it is necessary for the decorative sheet to be opaque and to be suitable for high quality printing. Barrier sheets are not normally used in this type of laminate since chipboard is normally of a lighter shade than core sheets and hence is more easily masked.

The paper which is used for making decorative sheets is known as plastic base surface paper. In addition to being opaque and suitable for printing, it must be absorbent so that it may easily be impregnated with resin during a single pass through an impregnating bath, which typically takes about 20 sec. The same applies to the overlay sheet if it is to be printed. The absorbency of plastic base surface paper, as measured by the Klemm method, is typically in the range 30 to 65 mm/10 min if for use in a high-pressure laminate, or in the range 25 to 45 mm1/10 min if for use in a low-pressure laminate (in the Klemm method a strip of paper 15 mm wide is suspended vertically with one end in a dish of the liquid concerned and the distance the liquid soaks up the paper in ten minutes is measured). The absorbency of an overlay sheet is typically in the higher part of the range quoted for plastic base surface paper for use in a high-pressure laminate. The absorbency of plastic base surface paper may also be quoted in terms of porisity as measured by a Gurley porosity tester, since porosity is related to speed of absorbency in this instance. Plastic base surface paper typically has a Gurley porosity (20 oz) in the range 10 to 25 sec/100 ml preferably 20 to 25 sec/100 ml, if for use in a high-pressure laminate, or in the range 15 to 50 sec/100 ml if for use in a low-pressure laminate, although values of 70 sec/100 ml or more are acceptable.

The requirement for plastic base surface paper and overlay paper to be absorbent results in a relatively rough paper surface which is not particularly suitable for high quality gravure printing. There are two main problems. First, the rough surface makes it difficult to obtain complete print coverage from every gravure cell. Second, the absorbent nature of the paper allows ink to penetrate into the sheet and print intensity is therefore reduced.

Despite these problems, plastic base surface and overlay paper can be printed to a high standard, provided larger quantities of ink are used than would be needed on a good printing surface or provided a lower absorbency is acceptable.

It might be thought that the above-described problems could be simply overcome by the application of a pigment coating such as is commonly used in the manufacture of high quality printing papers. However, such coatings enhance printability not only by increasing surface smoothness, which would be acceptable in plastic base surface and overlay papers, but also by decreasing absorbency to an extent which would not be acceptable in such papers. Pigment-coated art papers, for example, typically have a Klemm absorbency below 5 mm/10 minutes, which is well below that required in plastic base surface and overlay papers.

The use of pigment coatings on surface papers for use in decorative laminates was in fact proposed in GB-A-653531, GB-A-674149 and FR-A-1048836 (corresponding to GB-A-674149). GB-A-653531 refers to an impregnation time of 20 minutes, which is far in excess of the 20 second impregnation times now conventional. Since GB-A-674149 and FR-A-1048836 are closely related to GB-A-653531, it is to be supposed that the papers they disclose would likewise have unacceptably long empregnation times.

US-A-3798111 discloses the application of hard abrasion resistant pigments to a wet web for use as a surface paper, whilst the web is still on the wire of a papermaking machine, for example by means of a secondary headbox. The resulting dried paper is subsequently printed.

US-A-3578483 discloses the application to a surface paper of a discontinuous solvent-based pigment coating composition. The resulting web is subsequently printed.

It has now been found that, contrary to previous expectations in the art, the printability of plastic base surface and oerlay papers can be improved without unacceptably reducing the capacity of the paper to absorb impregnating resins by applying to the paper a continuous coating containing a pigment and a binder.

Accordingly, the present invention provides in a first aspect a process for the manufacture of a decorative laminate comprising the steps of:
(a) applying an aqueous liquid coating composition comprising a pigment and a binder to a surface of a previously formed and dried decorative laminate surface or overlay paper to produce a continuous coating;
(b) printing a desired pattern on said coated surface of said paper;
(c) impregnating the resulting printed paper with a thermosetting resin; and
(d) laminating the impregnated paper to a support therefor under conditions effective to cure the resin, thereby to produce said decorative laminate, characterised in that:
(e) the continuous coating on the surface of the decorative laminate surface or overlay paper has a coatweight when dry of up to 10 gm-²; and
(f) the resulting coated decorative laminate surface or overlay paper has a Gurley porosity (567 g) of about 10 to 70 sec/100 ml.

In a second aspect, the present invention provides a decorative laminate surface or overlay paper carrying a continuous coating composition comprising a pigment and a binder on a surface thereof at a coatweight of up to 10 gm-², said paper having a Gurley porosity of about 10 to 70 sec/100 ml and said pigment being kaolin, calcium carbonate, titanium dioxide or barium sulphate.

In order to ensure that the absorbency of the present plastic base surface or overlay paper is at a suitable level and that the surface smoothness of the coating is at an optimum level, the coatweight and the weight ratio of pigment to binder must be chosen carefully. The preferred dry coatweight is in the range of from 2.5 to 3 gm-². The weight ratio of pigment to binder in the coating is preferably in the range 5:1 to 1:1, more preferably from 2.5:1 to 3.5: 1. The Gurley porosity (567 g) of the coated paper is preferably in the range 20 to 50 sec/100 ml.

The pigment is preferably one having a Mohs' hardness of less than 7, for example kaolin, calcium carbonate in precipitated or ground form, titanium dioxide or barium sulphate. Pigments having a Mohs' hardness greater than 7, such as alumina or hydrated alumina, various natural or synthetic alumino-silicates or silica or silica gel may however be used. The binder may be starch, casein, latex, polyvinyl alcohol or an aminoplast or other cross-linking resin.

Preferably the liquid coating composition comprising the pigment and binder is applied by size press treatment, although other coating techniques may be used, for example air-knife coating. It will be appreciated that size press treatment normally results in a coating being applied to both surfaces of the paper web.

Once the decorative laminate surface or overlay paper has been coated it may be calendered before being impregnated.

The present plastic base surface of overlay paper enables an improvement in print quality to be obtained as a result of more complete ink transfer from the gravure cells and of less ink absorption. It also permits a reduction in ink usage for a print of specified quality, or, for the same ink usage affords a better print than would be obtained on the same paper if it were not coated.

The invention will now be described with reference to the following examples:

### Example 1

A sheet of plastic base surface paper having a grammage of 100 gm-² was size press coated with an aqueous coating containing a mixture of kaolin (supplied by English China Clays under the designation "Supreme"), esterified starch and mealmine-formaldehyde resin in a weight ratio of 3:1:0.001. The coating was then dried, the dry coatweight being 3 gm-^{2.} The absorbency of both the coated and the uncoated paper was found to be 30 mm/10 min. The Gurley porosity (567 g) of the coated paper was found to be 24 sec/100 ml, and that of the uncoated paper was 18 sec/100 ml.

Both the coated paper and a sample of uncoated plastic base surface paper were then printed with the same amount of ink using a gravure printing process. On examination of the printed papers, it was found that the optical reflectivity of the uncoated paper (as measured by an Elrepho opacimeter) was 20% whereas that of the coated paper was 10%. Both papers absorbed a sufficient amount of resin to make satisfactory laminates and the colour or shade of the unprinted surface of a laminate containing the coated paper was judged to be the same as that of a laminate . containing uncoated paper.

### Example 2

A sheet of plastic base surface paper having a grammage of 120 gm-² was size press coated with an aqueous coating containing a mixture of barium sulphate (precipitated), esterified starch and melamine formaldehyde resin in a weight ratio of 3: 1: 0.001. The coating was then dried and calendered, the dry coatweight being 7 gm-². The Gurley porosity (567 g) of the coated paper was found to be 26 sec/100 mi, and that of the uncoated paper was 14 sec/100 ml.

Both the coated paper and a sample of uncoated plastic base surface paper were then printed with the same amount of ink using a gravure printing process. On examination of the printed papers, it was found that the optical reflectivity of the uncoated paper (as measured by an Elrepho opacimeter) was 20% whereas that of the coated paper was 18%. Both papers absorbed a sufficient amount of resin to make satisfactory laminates and the colour or shade of the unprinted surface of a laminate containing the coated paper was judged to be the same as that of a laminate containing uncoated paper.

### Example 3

A sheet of plastic base surface paper having a grammage of 120 gm-² was size press coated with an aqueous coating containing a mixture of titanium dioxide (supplied by British Titan Products, under the designation ALF), esterified starch and melamine formaldehyde resin in a weight ratio of 3:1:0.001. The coating was then dried and calendered, the dry coatweight being 6.6 gm-². The Gurley porosity (567 g) of the coated paper was found to be 69 sec1100 ml, and that of the uncoated paper was 14 sec/100 ml.

Both the coated paper and a sample of uncoated plastic base surface paper were then printed with the same amount of ink using a gravure printing process. On examination of the printed papers, it was found that the optical reflectivity of the uncoated paper (as measured by an Elrepho opacimeter) was 20% whereas that of the coated paper was 17%. Both papers absorbed a sufficient amount of resin to make satisfactory laminates and the colour or shade of the unprinted surface of a laminate containing the coated paper was judged to be the same as that of a laminate containing uncoated paper.

### Example 4

A sheet of plastic base surface paper having a grammage of 120 gm-² was size press coated with an aqueous coating containing a mixture of calcium carbonate (under the designation Hyd- rocarb) esterified starch and melamine formaldehyde resin in a weight ratio of 3:1:0.001. The coating was then dried and calendered, the dry coatweight being 5.5 gm-². The Gurley porosity (567 g) of the coated paper was found to be 50 sec/100 ml, and that of the uncoated paper was 14 sec/100 ml.

Both the coated paper and a sample of uncoated plastic base surface paper were then printed with the same amount of ink using a gravure printing process. On examination of the printed papers, it was found that the optical reflectivity of the uncoated paper (as measured by an Elrepho opacimeter) was 20% whereas that of the coated paper was 17%. Both papers absorbed a sufficient amount of resin to make satisfactory laminates and the colour or shade of the unprinted surface of a laminate containing the coated paper was judged to be the same as that of a laminate containing uncoated paper.

## Claims

1. A process forthe manufacture of a decorative laminate comprising the steps of:
(a) applying an aqueous liquid coating composition comprising a pigment and a binder to a surface of a previously formed and dried decorative laminate surface or overlay paper to produce a continuous coating;
(b) printing a desired pattern on said coated surface of said paper;
(c) impregnating the reuslting printed paper with a thermosetting resin; and
(d) laminating the impregnated paper to a support therefor under conditions effective to cure the resin, thereby to produce said decorative laminate, characterised in that:
(e) the continuous coating on the surface of the decorative laminate surface or overlay paper has a coatweight when dry of up to 10 gm-²; and
(f) the resulting coated decorative laminate surface or overlay paper has a Gurley porosity (567 g) of about 10 to 70 sec/100 ml.

2. A process for the manufacture of a decorative laminate as claimed in claim 1 wherein the coating is applied to said surface of the previously formed and dried decorative laminate surface or overlay paper at a coatweight of 2.5 to 3 gm-².

3. A process for the manufacture of a decorative laminate as claimed in claim 1 wherein the Klemm absorbency of the plastic base surface paper is in the range 25 to 65 mm/10 min.

4. A process for the manufacture of a decorative laminate as claimed in claim 1 wherein the pigment has a Mohs' hardness of less than 7.

5. A process for the manufacture of a decorative laminate as claimed in claim 4 wherein the pigment is one of kaolin, calcium carbonate, titanium dioxide or barium sulphate.

6. A process for the manufacture of a decorative laminate as claimed in claim 1 wherein the weight ratio of pigment to binder is in the range 5:1 to 1:1.

7. A process forthe manufacture of a decorative laminate as claimed in claim 6 wherein the ratio of pigment to binder is in the range 2.5:1 to 3.5:1.

8. A process for the manufacture of a decorative laminate as claimed in claim 1 wherein the coating is applied by size press treatment.

9. A process for manufacture of a decorative laminate as claimed in claim 1 wherein the binder comprises starch, casein, latex, polyvinyl alcohol, or an aminoplast or other cross-linking resin.

10. A decorative laminate surface or overlay paper carrying a continuous coating composition comprising a pigment and a binder on a surface thereof at a coatweight of up to 10 gm-², said paper having a Gurley porosity (567 g) of about 10 to 70 sec/100 ml and said pigment being kaolin, calcium carbonate, titanium dioxide or barium sulphate.

11. A decorative laminate surface or overlay paper as claimed in claim 10 wherein said coating composition is present at a coatweight of 2.5 to 3 gₘ-2_{.}

12. A decorative laminate surface or overlay peper as claimed in claim 10 or 11 where the weight ratio of pigment to binder is in the range 5:1 to 1:1.

13. A decorative laminate surface or overlay paper as claimed in claim 12 wherein the weight ratio of pigment to binder is in the range 2.5:1 to 3.5:1.

## Revendications

1. Procédé pour la fabrication de stratifiés décoratifs comprenant les étapes consistant:
(a) à appliquer une composition liquide aqueuse de revêtement contenant un pigment et un liant sur une surface d'un papier enduit ou d'un papier de surface stratifiée décorative, préalablement formé et séché, en vue d'obtenir une couche de revêtement continu,
(b) à imprimer le motif désiré sur ladite surface revêtue dudit papier;
(c) à imprégner le papier imprimé résultant avec une résine thermodurcissable; et
(d) à stratifier le papier imprégné sur un support, dans des conditions permettant de durcir la résine et ainsi fournir ledit stratifié décoratif, caractérisé par le fait que:
(e) le poids de couche à sec du revêtement continu sur la surface du papier enduit ou du papier de surface stratifiée décorative est d'au plus 10 g/m-²; et que
(f) la porosité Gurley (567 g) du papier enduit ou du papier de surface stratifiée décorative ainsi couché est d'environ 10 à 70 sec/100 ml.

2. Procédé oour la fabrication de stratifiés décoratifs selon la revendication 1, caractérisé par le fait que le revêtement est appliqué à ladite surface du papier enduit ou du papier de surface stratifiée décorative, préalablement formé et séché, selon un poids de couche de 2,5 à 3 g/_{M}-².

3. Procédé pour la fabrication de stratifiés décoratifs selon la revendication 1, caractérisé par le fait que l'absorption Klemm du papier de surface pour base plastique est dans le domaine de 25 à 65 mm/10 min.

4. Procédé pour la fabrication de stratifié décoratif selon la revendication 1, caractérisé par le fait que le pigment a une dureté Moh inférieure à 7.

5. Procédé pour la fabrication de stratifiés décoratifs selon la revendication 4, caractérisé par le fait que le pigment est choisi parmi le kaolin, le carbonate de calcium, le dioxyde de titane ou le sulfate de baryum.

6. Procédé pour la fabrication de stratifiés décoratifs selon la revendication 1, caractérisé par le fait que le rapport en poids de pigment au liant est compris entre 5:1 et 1:1.

7. Procédé pour la fabrication de stratifiés décoratifs selon la revendication 6, caractérisé par le fait que le rapport du pigment au liant est compris entre 2,5:1 et 3,5:1.

8. Procédé pour la fabrication de stratifiés dédo- ratifs selon la revendication 1, caractérisé par le fait que le revêtement est appliqué par traitement à l'aide d'une presse encolleuse (ou "size press").

9. Procédé pour la fabrication de stratifiés décoratifs selon la revendication 1, caractérisé par le fait que le liant est choisi parmi l'amidon, la caséine, du latex, de l'alcool polyvinylique ou une résine aminoplaste ou toute autre résine réticulée.

10. Papier enduit ou de surface stratifiée décorative comportant une composition de revêtement continu contenant un pigment et un liant sur leur surface selon un poids de couche d'au plus 10 gtm-², ledit papier ayant une porosité Gurley (567 g) d'environ 10 à 70 sec/100 ml, et ledit pigment étant du kaolin, du carbonate de calcium, du dioxyde de titane ou du sulfate de baryum.

11. Papier enduit ou de surface stratifiée décorative selon la revendication 10, caractérisé par le fait que la composition de revêtement a un poids de couche de 2,5 à 3 g/m-².

12. Papier enduit ou de surface stratifiée décorative tel que revendiqué selon l'une quelconque des revendications 10 ou 11, caractérisé par le fait que le rapport en poids du pigment au liant est compris entre 5:1 et 1:1.

13. Papier enduit ou de surface stratifiée décorative tel que revendiqué selon la revendication 12, caractérisé par le fait que le rapport en poids du pigment au liant est compris entre 2,5:1 et 3,5:1.

## Patentansprüche

1. Verfahren zur Herstellung eines Dekorationsschichtstoffes bestehend aus den Schritten:
a) des Aufbringens einer flüssigen aus einem Pigment und einem Bindemittel bestehenden Beschichtungszusammensetzung auf einer Oberfläche einer zuvor geformten und getrockneten Dekorationsschichtstoffoberfläche oder eines Deckpapiers zur Erzeugung einer ununterbrochenen Beschichtung;
b) des Aufdruckens des gewünschten Musters auf diese beschichtete Oberfläche dieses Papiers;
c) des Imprägnierens des sich ergebenden bedruckten Papiers mit einem hitzehärtbaren Harz; und
d) des Beschichtens des imprägnierten Papiers auf einen Träger unter Bedingungen, bei welchem das Harz aushärtet, wobei dieser Dekorationsschichtstoff entsteht, dadurch gekennzeichnet, daß:
e) die ununterbrochene Beschichtung auf der Oberfläche der Dekorationsschichtstoffoberfläche oder des Deckpapiers ein Beschichtungsgewicht im trockenen Zustand von bis zu 10 gm-²; und
f) die sich ergebende beschichtete Dekorationsschichtstoffoberfläche oder das Deckpapier eine Gurley-Porosität (567 g) von etwa 10 bis 70 sec/ 100 ml aufweist.

2. Verfahren zur Herstellung eines Dekorationsschichtstoffs nach Anspruch 1, bei welchem die Beschichtung auf diese Oberfläche der zuvor geformten und getrockneten Dekorationsschichtstoffoberfläche oder des Deckpapiers mit einem Beschichtungsgewicht von 2,5 bis 3 gm-² aufgebracht wird.

3. Verfahren zur Herstellung eines Dekorationsschichtstoffs nach Anspruch 1, bei welchem die Klemm-Absorbierbarkeit des Oberfächenpapiers auf Kunstoffbasis im Bereich von 25 bis 65 mm/1 0 min liegt.

4. Verfahren zur Herstellung eines Dekorationsschichtstoffs nach Anspruch 1, bei welchem das Pigment eine Mohs-Härte von weniger als 7 aufweist.

5. Verfahren zur Herstellung eines Dekorationsschichtstoffs nach Anspruch 4, bei welchem das Pigment eines von Kaolin, Kalziumkarbonat, Titandioxyd oder Bariumsulfat ist.

6. Verfahren zur Herstellung eines Dekorationsschichtstoffs nach Anspruch 1, bei welchem das Gewichtsverhältnis von Pigment zu Bindemittel im Bereich von 5:1 bis 1:1 liegt.

7. Verfahren zur Herstellung eines Dekorationsschichtstoffs nach Anspruch 6, bei welchem das Verhältnis von Pigment zu Bindemittel im Bereich von 2,5:1 bis 3,5:1 liegt.

8. Verfahren zur Herstellung eines Dekorationsschichtstoffs nach Anspruch 1, bei welchem die Beschichtung durch Leimwerkbehandlung aufgebracht wird.

9. Verfahren zur Herstellung eines Dekorationsschichtstoffs nach Anspruch 1, bei welchem das Bindemittel aus Stärke, Kasein, Latex, Polyvinylalkohohl oder einem Aminoplast oder einem anderen vernetzten Harz besteht.

10. Dekorationsschichtstoffoberfläche oder Deckpapier, das auf einer seiner Oberflächen eine ununterbrochene Beschichtungszusammensetzung trägt, bestehend aus einem Pigment und einem Bindemittel mit einem Beschichtungsgewicht von bis zu 10 gm-², wobei dieses Papier eine Gurley-Porosität (567 g) von etwa 10 bis 70 sec/100 ml aufweist und das Pigment aus Kaolin, Kalziumkarbonat, Titandioxyd oder Bariumsulfat besteht.

11. Dekorationsschichtstoffoberfläche oder Deckpapier nach Anspruch 10, bei welchem die Beschichtungszusammensetzung mit einem -Beschichtungsgewicht von 2,5 bis 3 gm-² vorliegt.

12. Dekorationsschichtstoffoberfläche oder Deckpapier nach Anspruch 10 oder 11, bei welchem das Gewichtsverhältnis von Pigment zu Bindemittel im Bereich von 5:1 bis 1:1 liegt.

13. Dekorationsschichtstoffoberfläche oder Deckpapier nach Anspruch 12, bei welchem das Gewichtsverhältnis von Pigment zu Bindemittel im Bereich von 2,5:1 bis 3,5:1 liegt.
